# EUROPEAN PATENT SPECIFICATION

(11) **EP 1 651 801 B1**
(45) Date of publication and mention of the grant of the patent: **23.01.2008**
(21) Application number: 04763597.4
(22) Date of filing: 28.07.2004
(51) Int. Cl.: C25D 3/38

(54) **AQUEOUS, ACIDIC SOLUTION AND METHOD FOR ELECTROLYTICALLY DEPOSITING COPPER COATINGS AS WELL AS USE OF SAID SOLUTION**
WÄSSRIGE, SAURE LÖSUNG UND VERFAHREN ZUR ELEKTROLYTISCHEN ABSCHEIDUNG VON KUPFERÜBERZÜGEN SOWIE VERWENDUNG DER LÖSUNG
SOLUTION AQUEUSE ACIDE ET PROCEDE DE DEPOT ELECTROLYTIQUE DE REVETEMENTS DE CUIVRE, ET UTILISATION DE LADITE SOLUTION

(30) Priority: 08.08.2003 DE 10337669
(43) Date of publication of application: 03.05.2006
(73) Proprietor: ATOTECH Deutschland GmbH, 10553 Berlin (DE)
(72) Inventor: DAHMS, Wolfgang, 13437 Berlin (DE); FELS, Carl, Christian, 10115 Berlin (DE); BAUER, Günther, 14089 Berlin (DE)
(74) Representative: Patentanwälte Bressel und Partner
(86) International application number: PCT/EP2004/008492
(87) International publication number: WO 2005/014891

(56) References cited:
- EP-A- 1 001 054
- EP-A- 1 300 486
- EP-A- 1 300 487
- FR-A- 2 139 724
- US-A- 4 000 047
- US-A- 4 601 847

## Description

The present invention relates to an aqueous, acidic solution and to a method of electrolytically depositing copper coatings as well as to the use of said solution. Both solution and method preferably serve to produce high polish, decorative bright, smooth and level surfaces on large area metal or plastic parts as well as to coat printed circuit board material.

Various methods and deposition solutions are being used to produce decorative bright, smooth and level surfaces, more specifically large area surfaces, on metals or plastics or to form ductile layers such as for subsequent metallization.

To this day, acid copper electrolyte solutions, more specifically the widespread sulfuric acid copper electrolyte solutions, have been used for forming bright copper coatings. In order to avoid formation of undesirable crystalline matte deposits, small amounts of certain organic substances are added to these solutions. At first, for example cellulose, dextrine, gelatine, adhesive glue and molasses were used therefore, followed later by thiourea and the derivatives thereof, organic sulfides and quaternary nitrogen compounds. The relevant literature further mentions polyvinyl alcohol, organic phosphorus compounds and organic dyes like Janus green or crystal violet as additives (see "Kupferschichten - Abscheidung, Eigenschaften, Anwendung", (*"*Copper layers - deposition, properties, application"), N. Kanani, Leuze-Verlag, pages 93 and 76 and "Handbuch der Galvanotechnik" - ("Manual of Electroplating"), Dettner, Elze, Carl Hanser Verlag, vol. II, page 65).

In the light of the ever increasing demands that are placed on the quality of the metal layers and surfaces formed, these solutions have no importance whatsoever in today's practice since the quality of the copper coatings obtained using them does not meet today's requirements. For these coatings are either too brittle or not bright enough or, in certain current density ranges, the coatings obtained show a kind of relief.

Various other solutions have been tested to meet the new requirements. It has become known to add polyalkylene imines in combination with organic thio compounds (DE 1 246 347 A) and polyvinyl compounds in combination with oxygen-containing high molecular compounds and organic, more specifically aromatic, thio compounds (DE 1 521 062 A). Such type copper electrolyte solutions do not allow for utilization of higher cathodic current densities, though. Another disadvantage is that the deposited copper coatings must be subjected to an intermediate treatment prior to being metal plated, e.g., nickel-plated.

DE 1 521 062 A describes an acidic copper bath that contains, in addition to an oxygen-containing polymeric compound, at least one substituted phenazinium compound.

Using the described monomeric phenazinium compounds in copper plating electrolytes, problems arise in practicing the process. It has been recognized that the current density that may be applied as well as the aging behavior of the deposited metal layers may still be optimized.

Combinations of organic thio compounds and non-ionogenic wetting agents with other dyes such as crystal violet (EP 0 071 512 A1), amides (DE 27 46 938 A1) or phthalocyanine derivatives with aposafranine (DE 34 20 999 A1) are further used for depositing copper.

Further EP 1 300 486 A1 and EP 1 300 487 A1 disclose metal plating baths, more specifically copper plating baths, which comprise additive consumption inhibiting aldehyde or alcohol, respectively. Among a multitude of expressly disclosed aldehydes or alcohols, respectively, 2-chloro-4-hydroxybenzaldehyde as well as 4-chlororesorcinol, α,α,α-trifluoro-*m*-cresol and 3-chlorophenol are mentioned exemplarily. The aldehydes or alcohols are comprised in the baths at a concentration of 0.001 -100 g/l. Examples show that these compounds are contained at a concentration of 1 g/l.

Undefined reaction products of polyamines with benzyl chloride (DE 25 41 897 A1) or with epichlorohydrin (EP 0 068 807 A1), respectively, or reaction products with thio compounds and acrylamide (EP 0 107 109 A1) are also used in lieu of the dye.

The major disadvantage of the last mentioned solutions, more specifically when combined with nitrogen-containing thio compounds, is non-uniform deposition of the copper layer onto the surface of a substrate.

DE 20 39 831 C describes how the quality of the metal surfaces deposited may be enhanced using polymeric phenazinium compounds. In the plating bath, these polymeric phenazinium compounds are mainly utilized in combination with non-ionogenic wetting agents and organic sulfur compounds.

A prerequisite of producing smooth surfaces is that the solution permits high leveling of the surface to be coated. High leveling however yields surfaces having a disadvantageous fine roughness (pittings, nodules) that severely affects the decorative appearance of large area parts in particular.

It has been recognized that this roughness is not due to particles suspended in the electrolyte as such a roughness could not be readily avoided by filtering the electrolyte. The fine roughness that forms with high leveling is due to a spontaneously disturbed deposition-which is also discussed to be a disguised whisker formation - in the cathodic double layer and particularly occurs with thicker copper layers having a thickness in excess of 5 µm. A corresponding defect may be recognized in the polished cross section of the metal layer deposited, said defect becoming apparent in the form of nodules or pittings on the surface as the other layers are being deposited. These pittings and nodules are particularly apparent on polished large area steel and plastic parts where the mirror-bright polish of the deposit even further emphasizes this effect.

This phenomenon was particularly observed using nitrogen-containing sulfur compounds (thiourea derivatives) and phenazinium compounds in plating electrolyte solutions. To circumvent this drawback DE 40 32 864 A1 discloses the use of special non-ionogenic wetting agents, in the present case more specifically of naphthol ethoxylates.

It has been recognized though that, when used in effective concentrations, the naphthol ethoxylates result in disturbing anode effects such that the anode film may completely come off or that the anode dissolves non-uniformly, which is not desirable.

Accordingly, using the known methods and treatment solutions, it is not possible to produce decorative bright and level metal surfaces that have no undesirable effects such as pittings and nodules. Using the known solutions, it is not possible to achieve high leveling without compromising the bright appearance of the surface layer. Moreover, both solution and method are intended to save costs and their process reliability must be high.

It is therefore the object of the present invention to avoid the prior art drawbacks. The invention more specifically aims at providing a solution and a method of deposition that permit advantageous high leveling of the surface to be coated while concurrently preventing fine roughness from forming, so that decorative bright metal surfaces may be formed on metal or plastic substrates and ductile metal layers on printed circuit board material.

In overcoming these problems, the invention provides the solution for depositing copper coatings in accordance with claim 1, the method in accordance with claim 24 and the use of the solution in accordance with claims 21 and 22. Preferred embodiments of the invention will become apparent in the dependant claims.

The solution of the invention is an aqueous acidic solution (electrolyte solution) and serves to electrolytically deposit bright copper coatings in particular, preferably decorative bright copper coatings, on large area metal or plastic parts such as in the automobile, the furniture or the sanitary industry, *e.g*., for metallizing automobile bumpers or shower heads as well as to deposit copper on printed circuit board material. The solution of the invention

is as defined in claim 1.

If several radicals are halogen, the preferred number of radicals R₁, R₂, R₃, R₄, R₅ and R₆ which may be halogen ranges from one to three, more preferably from one to two. One halogen is most preferred.

The amount of the at least one aromatic halogen derivative, or of the salt thereof respectively, that is to be added to significantly improve copper deposition is extremely low. The concentration thereof ranges from 0.005 to 0.9 mg/l, more preferably from 0.005 to 0.5 mg/l, a concentration of 0.02 or more being particularly preferred, a concentration of 0.3 mg/l or less being even more preferred and a concentration in the range of from 0.02 to 0.2 mg/l being most preferred.

Surprisingly, fine roughness could be prevented from forming using but small amounts of aromatic halogen derivatives. The proof of the effectiveness of the copper deposition can be furnished using cyclic voltammetry. The addition in accordance with the invention of aromatic halogen derivatives inhibits copper deposition, which becomes apparent as the stripping peak shifts toward anodic potentials. In addition, by adding aromatic halogen derivatives, the quotient of the anodic charge in the dissolution area (stripping peak) and of the cathodic charge in the deposition area (plating peak) increases from 93 to 100 %. High polish leveled copper coatings (without any nodules and pittings) are produced as a result thereof.

Whereas the aromatic halogen derivatives having hydroxy groups at the aromatic compound (halogen phenol derivatives) act spontaneously, the action of the aldehydic substituted aromatic halogen derivatives is slightly delayed. This points to the fact that the hydroxy compounds constitute the active substances and that they can also be formed in the solution by reducing the aldehyde derivatives. Such theoretic considerations will not affect the scope of the invention, though. The structure of the copper crystallites on the surface to be coated changes during deposition. The grain boundaries formed are finer and the crystallites are generally smaller.

The method in accordance with the invention is simple, easy to perform and cheap. It serves to deposit high polish copper coatings on metal or plastic surfaces, the surfaces being brought into contact with the solution of the invention and copper being electrolytically deposited onto the surfaces.

The metal or plastic surfaces to be coated preferably include large area surfaces pertaining for example to the field of the automobile, toy, furniture or sanitary industry. The bright copper coatings more specifically serve decorative purposes, for example on coated automobile bumpers, automobile spoilers or wind deflectors, toys, shower heads, towel racks, and so on.

The metal or plastic surfaces also include surfaces of printed circuit boards. In this field, throwing power improves using both direct current and pulsed current for copper deposition.

The solution in accordance with the invention and the method permit to eliminate the problems arising using the known means. They more specifically permit to form high polish, decorative surfaces on metal and plastic surfaces while avoiding the formation of quality impairing effects such as nodules and pittings. Concurrently, besides high leveling, fine roughness is prevented from forming.

In order to achieve, for the solution of the invention, the deposition effect described, the aromatic halogen derivatives each independently contain substituted radicals. The radicals R₁, R₂, R₃, R₄, R₅ and R₆ present at the aromatic halogen derivatives may concurrently be the same and different.

Halogen is preferably selected from the group comprising fluorine, chlorine, bromine and iodine, with chlorine and bromine being particularly preferred.

The aldehyde radicals are thereby preferably selected from the group comprising formyl (-CHO), methylformyl (-CH₂-CHO) and ethylformyl (-C₂H₄-CHO).

The alkyl radicals are preferably selected from the group of branched and unbranched carbon chains having 1 -4 carbon atoms, comprising methyl, ethyl, *n*-propyl, *iso*-propyl, *n*-butyl, *iso*-butyl and *tert*-butyl.

The hydroxyalkyl radicals preferably comprise branched or unbranched carbon chains having 1-4 carbon atoms, corresponding to the previously mentioned carbon chains of the alkyl radicals mentioned hereinbefore, each of the alkyl radicals mentioned hereinbefore containing at least one hydroxy group. Preferably, at least one hydroxyalkyl radical is a hydroxymethyl.

If the aromatic halogen derivatives according to the general formula (I) are used in the solution of the invention, the following compounds are particularly suited.

Aromatic Halogen Derivatives:
2-chlorobenzaldehyde
2-chlorophenol
4-chloro-3-methylphenol
2-chloro-4,5-dimethylphenol
4-chloro-3,5-dimethylphenol
4-chlorophenol
3-chlorophenol
o- chloroacetophenone
2-chlorobenzyl alcohol
4-bromo-2,6-dimethylphenol
4-bromophenol
2,4-dichlorobenzyl alcohol
2,6-dibromo-4-methylphenol
2,5-dichlorophenol
3,5-dibromobenzaldehyde
2,5-dibromobenzoic acid
2,4,6-trichlorophenol
2,3,6-trichlorobenzaldehyde

Before use, the aromatic halogen derivatives are preferably dissolved in methanol or in other alcohols (e.g., glycol) or polyalcohols (e.g., polyethylene glycol) and then added to the solution of the invention. To dissolve the aromatic halogen derivatives in the solution of the invention, it is often helpful to alkalinize the solution, certain amounts of salts that are readily soluble in water such as alkali halogen phenolates forming in the process. A bisulfite adduct forming with the CO-group of the aldehyde radical may also be used to improve water solubility with, possibly, partial formation of α-hydroxysulfonates. Partial acetal formation may also occur if aldehyde-containing aromatic halogen derivatives are dissolved in alcohol.

The aromatic halogen derivatives are actually known and are mostly commercially available or may be produced according to known methods.

The current brighteners, wetting agents or levellers also enhance other physical properties such as the ductility of the layers for example. Examples of these compounds are oxygen-containing, high molecular additives and water soluble sulfur compounds.

The at least one oxygen-containing high molecular additive contained in the solution of the invention is a polyalkylene glycol compound, for example a polyalkylene glycol or an acid ester, more specifically carboxylic acid ester or alcohol ether, such as alkanol ether or phenol ether, of a polyalkylene glycol. The additive is more specifically selected from the group comprising

Oxygen-containing high molecular additives:
polyvinyl alcohol
carboxymethyl cellulose
polyethylene glycol
polypropylene glycol
stearic acid polyglycol ester
oleic acid polyglycol ester
stearyl alcohol polyglycol ether
nonylphenol-polyglycol ether
octanol polyalkylene glycol ether
octanediol-bis-(polyalkylene glycol ether)
poly(ethylene glycol-*ran*-propylene glycol)
poly(ethylene glycol)-*block*-poly(propylene glycol)-*block* poly(ethylene glycol)
poly(propylene glycol)-*block*-poly(ethylene glycol)-*block-*poly(propylene glycol)

The amount of the at least one oxygen-containing high molecular additive preferably corresponds to a concentration range of from 0.005 to 20 g/l, more preferably to a concentration range of from 0.01 to 5 g/l.

The at least one water soluble sulfur compound contained in the solution of the invention is preferably selected from the group comprising organic, nitrogen-free thio compounds and the salts thereof. The salts preferably contain alkali or earth alkali metal ions, selected from the group comprising sodium, potassium, magnesium and calcium.

The salts of the following organic nitrogen-free thio compounds are particularly suited:

Organic nitrogen-free thio compounds:
sodium salt of 3-(benzthiazolyl-2-thio)-propylsulfonic acid
sodium salt of 3-mercaptopropane-1-sulfonic acid
disodium salt of thiophosphoric acid-O-ethyl-bis-(ω-sulfopropyl)-ester
trisodium salt of thiophosphoric acid-tris-(ω-sulfopropyl)-ester
sodium salt of ethylenedithio dipropyl sulfonic acid
disodium salt of bis-(*p*-sulfophenyl)-disulfide
disodium salt of bis-(ω-sulfopropyl)-sulfide
disodium salt of bis-(ω-sulfopropyl)-disulfide
disodium salt of bis-(ω-sulfohydroxypropyl)-disulfide
disodium salt of bis-(ω-sulfobutyl)-disulfide
sodium salt of methyl-(ω-sulfopropyl)-disulfide
sodium salt of methyl-(ω-sulfobutyl)-trisulfide
potassium salt of O-ethyl-dithiocarbonic acid-S-(ω-sulfopropyl)-ester thioglycolic acid.

The amount of the at least one water soluble sulfur compounds or of the salts thereof preferably corresponds to a concentration range of from 0.0005 to 0,4 g/l, more preferably to a concentration range of from 0.001 to 0,15 g/l.

The solution of the invention further contains at least one acid. Said acid is preferably selected from the group comprising sulfuric acid, hydrochloric acid, fluoboric acid and methanesulfonic acid.

The amount of the at least one acid, preferably of the sulfuric acid, preferably corresponds to a concentration range of from 50 to 350 g/l, more preferably to a concentration range of from 180 to 220 g/l or of from 50 to 90 g/l.

The solution of the invention may additionally contain chloride ions. The chloride ions are preferably added to the solution in the form of sodium chloride and/or of hydrochloric acid. The addition of sodium chloride may be dispensed with in part or in whole if chloride ions are already contained in other additives.

The copper ions needed for depositing copper coatings are provided either by copper salts, preferably copper sulfate, or by soluble copper anodes, which are preferably located in the conventional anode baskets inside or outside of the solution. Copper ions may also be supplied to the solution by chemically dissolving small pieces of copper in a separate container using atmospheric oxygen or iron(III) ions.

The basic composition of the solution of the invention may vary over wide limits as indicated. As a result and in addition to the concentration ranges given for the oxygen-containing high molecular additives, the water soluble sulfur compounds, the acids, preferably the sulfuric acid, and the aromatic halogen derivatives, the aqueous acidic solution of the invention generally further contains: copper sulfate (CuSO₄ · 5 H₂O) in a concentration range of preferably from 20 to 250 g/l, more preferably of from 60 to 80 g/l or from 180 to 220 g/l and chloride ions in a concentration range of preferably from 0.02 to 0.25 g/l, more preferably of from 0.05 to 0.12 g/l.

Other copper salts than copper sulfate may be used in part. The sulfuric acid can also be replaced, in part or in whole, with fluoboric acid, methanesulfonic acid, hydrochloric acid or by other acids.

In order to further enhance levelling of the surfaces to be coated, the solution of the invention may contain other additional levellers either together or individually. At least one nitrogen-containing thio compound, at least one polymeric phenazinium compound and/or at least one polymeric nitrogen compound are preferably added to the solution of the invention.

Particularly suited nitrogen-containing thio compounds are:

Nitrogen-containing thio compounds (thiourea derivatives):
thiourea
N-acetylthiourea
N-trifluoroacetyl thiourea
N-ethylthiourea
N-cyanoacetyl thiourea
N-allylthiourea
o-tolylthiourea
N,N'-butylene thiourea
thiazolidine thiol-2
4-thiazoline thiol-2
imidazolidine thiol-2-(N,N'-ethylene thiourea)
4-methyl-2-pyrimidine thiol
2-thiouracil

The amount of the at least one nitrogen-containing thio compound preferably corresponds to a concentration range of from 0.0001 to 0.5 g/l, more preferably to a concentration range of from 0.005 to 0.04 g/l.

Particularly suited polymeric phenazinium compounds are:

Polymeric phenazinium compounds:
poly(6-methyl-7-dimethylamino-5-phenyl-phenazinium sulfate)
poly(2-methyl-7-diethylamino-5-phenyl-phenazinium chloride)
poly(2-methyl-7-dimethylamino-5-phenyl-phenazinium sulfate)
poly(5-methyl-7-dimethylamino-phenazinium acetate)
poly(2-methyl-7-anilino-5-phenyl-phenazinium sulfate)
poly(2-methyl-7-dimethylamino-phenazinium sulfate)
poly(7-methylamino-5-phenyl-phenazinium acetate)
poly(7-ethylamino-2,5-diphenyl-phenazinium chloride)
poly(2,8-dimethyl-7-diethylamino-5-*p*-tolyl-phenazinium chloride)
poly(2,5,8-triphenyl-7-dimethylamino-phenazinium sulfate)
poly(2,8-dimethyl-7-amino-5-phenyl-phenazinium sulfate)
poly(7-dimethylamino-5-phenyl-phenazinium chloride)

The amount of the at least one polymeric phenazinium compound preferably corresponds to a concentration range of from 0.0001 to 0.5 g/l, more preferably to a concentration range of from 0.005 to 0.04 g/l.

Particularly suited polymeric nitrogen compounds are:

Polymeric nitrogen compounds:
polyethylene imine
polyethylene imide
polyacrylic acid amide
polypropylene imine
polybutylene imine
N-methyl polyethylene imine
N-acetyl polyethylene imine
N-butyl polyethylene imine

The amount of the at least one polymeric nitrogen compound preferably corresponds to a concentration range of from 0.0001 to 0.5 g/l, more preferably to a concentration range of from 0.005 to 0.04 g/l.

In a preferred embodiment, the solution of the invention may contain, in addition to the basic composition described, oxygen-containing, high molecular additives, water soluble sulfur compounds, acids, copper sulfate, chloride ions and aromatic halogen derivatives, at least one of the nitrogen-containing thio compounds mentioned hereinbefore, at least one of the polymeric phenazinium compounds mentioned hereinbefore and at least one of the polymeric nitrogen compounds mentioned hereinbefore.

The electrolytic deposition of copper coatings is preferably performed under the following conditions:

| | |
|---|---|
| pH-value: | < 1; |
| temperature: | from 15 to 50°C, |
| more preferably | from 20 to 33°C; |
| cathodic current density: | from 0.5 to 12 A/dm², |
| more preferably | from 2 to 4 A/dm². |

Sufficient mixing of the solution of the invention during deposition is achieved by a strong flow and, at need, by blowing clean air into the mixture so that the surface of the solution is strongly agitated. As a result, the transport of substances in proximity to the electrodes is maximized, which makes it possible to achieve higher current densities. It is moreover possible to enhance the transport of substances at the respective surfaces by causing the cathodes to move. Thanks to the thus increased convection and to the movement of the electrodes, constant, diffusion-controlled deposition is performed. The electrodes may be moved horizontally, vertically and/or by vibration or ultrasound for example. This is particularly effective in combination with air being blown in.

The copper content of the solution of the invention can be electrochemically replenished, during deposition, using soluble copper anodes. The anode material used is preferably copper containing 0.02- 0.06 % phosphorus (m/m). In order to prevent dirt accumulation on the copper anodes, they should be sealed from the electrolyte by anode bags. Inert anodes may be used in the alternative. In this case, the copper content must be replenished from a separate dissolution compartment.

In order to maintain the quality of the solution of the invention, filters for retaining mechanical and/or chemical residues may be inserted into the solution's circulation system. If soluble copper anodes are used, filtration is highly recommended because the phosphorus causes anode sludge to form which can disturb the deposition process. Using inert anodes, the quality of the solution may be maintained at less expense.

The work piece can be coated in horizontal or vertical conveyorized plating lines.

The following examples serve to explain the invention:

### Comparative Example 1a:

An aqueous acidic solution was prepared by mixing the following constituents:

| | |
|---|---|
| copper sulfate (CuSO₄· 5 H₂O) | 200.0 g |
| sulfuric acid (96 % (m/m)) | 65.0 g |
| sodium chloride | 0.2 g |
| polyethylene glycol | 0.2 g |
| disodium salt of bis-(ω-sulfopropyl)-disulfide | 0.01 g |
| 7-dimethylamino-5-phenyl-phenazinium chloride (polymer) and deionized water to bring the volume to 1 l. | 0.02 g |

The solution was heated to 27°C. Then, in accordance with the method of the invention a polished brass plate was brought into contact with the solution.

Cathodic current density was 4 A/dm². During deposition, air was blown into the solution in order to achieve thorough mixing.

A well-leveled bright copper coating appeared on the brass plate which, on closer examination, showed fine roughness (pittings), though.

### Example 1 b - Example in accordance with the invention

Comparative Example 1 a was repeated with the same solution, except that the following aromatic halogen derivative was now added in accordance with the invention:

| | |
|---|---|
| 4-chloro-3,5-dimethylphenol | 0.1 mg |

Deposition resulted in a well-leveled, mirror polish copper coating. The coating showed no voids.

### Comparative Example 1 c

Comparative Example 1 a was repeated. 76 mg/l of 4-chloro-3,5-dimethylphenol were added to the deposition solution. The deposit produced was not bright but rather had a mist-type appearance being comprised of a plurality of pittings and nodules.

### Comparative Example 1d

Comparative Example 1 a was repeated. 152 mg/l of 4-chloro-3,5-dimethylphenol were added to the solution. The deposit was matte and could therefore not be used as a decorative coating.

### Comparative Example 2a

An aqueous acidic solution was prepared by mixing the following constituents:

| | |
|---|---|
| copper sulfate (CuSO₄· 5 H₂O) | 80.0 g |
| sulfuric acid (96 % (m/m)) | 180.0 g |
| sodium chloride | 0.08 g |
| polypropylene glycol | 0.6 g |
| sodium salt of 3-mercaptopropane-1-sulfonate | 0.02 g |
| N-acetylthiourea | 0.003 g |
| and deionized water to bring the volume to 1 l. | |

The solution was heated to 30°C. Then, in accordance with the method of the invention a brushed copper laminate was brought into contact with the solution. Cathodic current density was 2 A/dm². During deposition, air was blown into the solution In order to achieve thorough, mixing.

On the copper laminate there appeared a bright copper coating which however showed fine roughness (pittings and nodules).

### Example 2b - Example In accordance with the Invention

Comparative Example 2a was repeated with the same solution, except that the following aromatic halogen derivative was now added in accordance with the invention:

| | |
|---|---|
| 2-chlorobenzaldehyde | 0.5 mg |

Deposition resulted in a well-leveled, mirror polish copper coating. The coating showed no voids.

## Claims

1. An aqueous acidic solution for electrolytically depositing copper coatings, said solution containing at least one polyalkylene glycol compound and at least one water soluble sulfur compound, **characterized in that** the solution additionally contains at least one aromatic halogen derivative having the general formula (I) wherein
R₁, R₂, R₃, R₄, R₅ and R₆ are each independently radicals selected from the group comprising hydrogen, aldehyde, acetyl, hydroxy, hydroxyalkyl having 1 - 4 carbon atoms, alkyl having 1-4 carbon atoms and halogen, with the proviso that the number of radicals R₁, R₂, R₃, R₄, R₅ and R₆ which are halogen ranges from 1 - 5 and that at least one of R₁, R₂, R₃, R₄, R₅ and R₆ is selected from the group consisting of hydroxy, aldehyde, acetyl and hydroxyalkyl having 1-4 carbon atoms, wherein the concentration of the at least one aromatic halogen derivative ranges from 0.005 - 0.9 mg/l.

2. The solution according to any one of the preceding claims, **characterized in that** the aldehyde is selected from the group comprising formyl (-CHO), methylformyl (-CH₂-CHO) and ethylformyl (-C₂H₄-CHO).

3. The solution according to any one of the preceding claims, **characterized in that** alkyl is branched or unbranched and is selected from the group comprising methyl, ethyl, *n*-propyl, *iso*-propyl, *n*-butyl, *iso*-butyl and *tert*-butyl.

4. The solution according to any one of the preceding claims, **characterized in that** alkyl is hydroxyalkyl and that it is branched or unbranched.

5. The solution according to any one of the preceding claims, **characterized in that** at least one hydroxyalkyl is hydroxymethyl.

6. The solution according to any one of the preceding claims, **characterized in that** the at least one aromatic halogen derivative is selected from the group comprising
2-chlorobenzaldehyde
2-chlorophenol
4-chloro-3-methylphenol
2-chloro-4,5-dimethylphenol
4-chloro-3,5-dimethylphenol
4-chlorophenol
3-chlorophenol
o-chloroacetophenone
2-chlorobenzyl alcohol
4-bromo-2,6-dimethylphenol
4-bromophenol
2,4-dichlorobenzyl alcohol
2,6-dibromo-4-methylphenol
2,5-dichlorophenol
3,5-dibromobenzaldehyde
2,5-dibromobenzoic acid
2,4,6-trichlorophenol
2,3,6 trichlorobenzaldehyde.

7. The solution according to any one of the preceding claims, **characterized in that** the at least one oxygen-containing, high molecular additive is selected from the group comprising
polyvinyl alcohol
carboxymethyl cellulose
polyethylene glycol
polypropylene glycol
stearic acid polyglycol ester
oleic acid polyglycol ester
stearyl alcohol polyglycol ether
nonylphenol-polyglycol ether
octanol polyalkylene glycol ether
octanediot-bis-(polyalkylene glycol ether)
poly(ethylene glycol-*ran*-propylene glycol)
poly(ethylene glycol)-*block*-poly(propylene glycol)-*block*-poly(ethylene glycol) and
poly(propylene glycol)-*block*-poly(ethylene glycol)-*block*-poly(propylene glycol).

8. The solution according to any one of the preceding claims, **characterized in that** the at least one water soluble sulfur compound is selected from the group comprising organic, nitrogen-free thio compounds and the salts thereof.

9. The solution according to claim 8, **characterized in that** the salts contain alkali or earth alkali metal ions, selected from the group comprising sodium, potassium, magnesium and calcium

10. The solution according to any one of claims 8 and 9, **characterized in that** the at least one organic nitrogen-free thio compound is selected from the group comprising
sodium salt of 3-(benzthiazolyl-2-thio)-propylsulfonic acid
sodium salt of 3-mercaptopropane-1-suifonic acid
disodium salt of thiophosphoric acid-O-ethyl-bis-(ω-sulfopropyl)-ester
trisodium salt of thiophosphoric acid-tris-(ω-sulfopropyl)-ester
sodium salt of ethylenedithio dipropyl sulfonic acid
disodium salt of bis-(*p*-sulfophenyl)-disulfide
disodium salt of bis-(ω-sulfopropyl)-sulfide
disodium salt of bis-(*p*-sulfopropyl)-disulfide
disodium salt of bis-(ω-sulfohydroxypropyl)-disulfide
disodium salt of bis-(ω-sulfobutyl)-disulfide
sodium salt of methyl-(ω-sulfopropyl)-disulfide
sodium salt of methyl-(ω-sulfobutyl)-trisulfide
potassium salt of O-ethyl-dithiocarbonic acid-S-(ω-sulfopropyl)-ester thioglycolic acid

11. The solution according to any one of the preceding claims, **characterized in that** acid is contained in the solution and that the acid is selected from the group comprising sulfuric acid, hydrochloric acid, fluoboric acid and methanesulfonic acid.

12. The solution according to any one of the preceding claims, **characterized in that** the solution additionally contains chloride ions.

13. The solution according to claim 12, **characterized in that** the chloride ions have been added to the solution in the form of sodium chloride and/or of hydrochloric acid.

14. The solution according to any one of the preceding claims, **characterized in that** the solution additionally contains at least one organic, nitrogen-containing thio compound.

15. The solution according to claim 14, **characterized in that** the at least one nitrogen-containing thio compound is selected from the group comprising
thiourea
N-acetylthiourea
N-trifluoroacetyl thiourea
N-ethylth iou rea
N-cyanoacetyl thiourea
N-allylthiourea
*o*-tolylthiourea
N,N'-butylene thiourea
thiazolidine thiol-2
4-thiazoline thiol-2
imidazolidine thiol-2-(N,N'-ethylene thiourea)
4-methyl-2-pyrimidine thiol
2-thiouracil

16. The solution according to any one of the preceding claims, **characterized in that** the solution additionally contains at least one polymeric phenazinium compound.

17. The solution according to claim 16, **characterized in that** the at least one polymeric phenazinium compound is selected from the group comprising
poly(6-methyl-7-dimethylamino-5-phenyl-phenazinium sulfate)
poly(2-methyl-7-diethylamino-5-phenyl-phenazinium chloride)
poly(2-methyl-7-dimethylamino-5-phenyl-phenazinium sulfate)
poly(5-methyl-7-dimethylamino-phenazinium acetate)
poly(2-methyl-7-anilino-5-phenyl-phenazinium sulfate)
poly(2-methyl-7-dimethylamino-phenazinium sulfate)
poly(7-methylamino-5-phenyl-phenazinium acetate)
poly(7-ethylamino-2,5-diphenyl-phenazinium chloride)
poly(2,8-dimethyl-7-diethylamino-5-*p*-tolyl-phenazinium chloride)
poly(2,5,8-triphenyl-7-dimethylamino-phenazinium sulfate)
poly(2,8-dimethyl-7-amino-5-phenyl-phenazinium sulfate)
poly(7-dimethylamino-5-phenyl-phenazinium chloride)

18. The solution according to any one of the preceding claims, **characterized in that** the solution additionally contains at least one polymeric nitrogen compound.

19. The solution according to claim 18, **characterized in that** the at least one polymeric nitrogen compound is selected from the group comprising polyethylene imine, polyethylene imide, polyacrylic acid amide, polypropylene imine, polybutylene imine, N-methyl polyethylene imine, N-acetyl polyethylene imine, N-butyl polyethylene imine.

20. Use of the solution according to any one of claims 1 - 19 for depositing a copper coating.

21. Use of the solution according to claim 20 for depositing copper onto printed circuit board material.

22. Use according to any one of claims 20 and 21 for producing copper coatings in vertical and/or horizontal conveyorized plating lines.

23. A method of electrolytically depositing copper coatings on metal or plastic surfaces, comprising bringing the surfaces into contact with the solution according to any one of claims 1 - 19 and electrolytically depositing copper onto the surfaces.

## Patentansprüche

1. Wässrige saure Lösung zum galvanischen Abscheiden von Kupferüberzügen, enthaltend mindestens eine Polyalkylenglykol-Verbindung und mindestens eine wasserlösliche Schwefelverbindung, **dadurch gekennzeichnet, dass** die Lösung zusätzlich mindestens ein aromatisches Halogenderivat mit der allgemeinen Formel (I) enthält: wobei
R₁, R₂, R₃, R₄, R₅ und R₆ jeweils unabhängig voneinander Reste sind, die ausgewählt sind aus der Gruppe, umfassend Wasserstoff, Aldehyd, Acetyl, Hydroxy, Hydroxyalkyl mit 1 - 4 Kohlenstoffatomen, Alkyl mit 1 - 4 Kohlenstoffatomen und Halogen, mit der Maßgabe, dass die Anzahl der Reste R₁, R₂, R₃, R₄, R₅ und R₆, welche Halogen sind, im Bereich von 1 - 5 liegt und dass mindestens einer der Reste R₁, R₂, R₃, R₄, R₅ und R₆ ausgewählt ist aus der Gruppe, bestehend aus Hydroxy, Aldehyd, Acetyl und Hydroxyalkyl mit 1 - 4 Kohlenstoffatomen, wobei die Konzentration des mindestens einen aromatischen Halogenderivats im Bereich von 0,005 - 0,9 mg/l liegt.

2. Lösung nach einem der vorstehenden Ansprüche, **dadurch gekennzeichnet, dass** der Aldehyd ausgewählt ist aus der Gruppe, umfassend Formyl (-CHO), Methylformyl (-CH₂-CHO) und Ethylformyl (-C₂H₄-CHO).

3. Lösung nach einem der vorstehenden Ansprüche, **dadurch gekennzeichnet, dass** Alkyl verzweigt oder unverzweigt ist und aus der Gruppe ausgewählt ist, umfassend Methyl, Ethyl, *n*-Propyl, *iso*-Propyl, *n*-Butyl, *iso*-Butyl und *tert*-Butyl.

4. Lösung nach einem der vorstehenden Ansprüche, **dadurch gekennzeichnet, dass** Alkyl Hydroxyalkyl ist und dass es verzweigt oder unverzweigt ist.

5. Lösung nach einem der vorstehenden Ansprüche, **dadurch gekennzeichnet, dass** mindestens ein Hydroxyalkyl Hydroxymethyl ist.

6. Lösung nach einem der vorstehenden Ansprüche, **dadurch gekennzeichnet, dass** das mindestens eine aromatische Halogenderivat ausgewählt ist aus der Gruppe, umfassend:
2-Chlorbenzaldehyd
2.-Chlorphenol
4-Chlor-3-methylphenol
2-Chlor-4,5-dimethylphenol
4-Chlor-3,5-dimethylphenol
4-Chlorphenol
3-Chlorphenol
*o*-Chloracetophenon
2-Chlorbenzylalkohol
4-Brom-2,6-dimethylphenol
4-Bromphenol
2,4-Dichlorbenzylalkohol
2,6-Dibrom-4-methylphenol
2,5-Dichlorphenol
3,5-Dibrombenzaldehyd
2,5-Dibrombenzoesäure
2,4,6-Trichlorphenol
2,3,6-Trichlorbenzaldehyd

7. Lösung nach einem der vorstehenden Ansprüche, **dadurch gekennzeichnet, dass** der mindestens eine sauerstoffhaltige, hochmolekulare Hilfsstoff ausgewählt ist aus der Gruppe, umfassend
Polyvinylalkohol
Carboxymethylcellulose
Polyethylenglykol
Polypropylenglykol
Stearinsäure-Polyglykolester
Ölsäure-Polyglykolester
Stearylalkohol-Polyglykolether
Nonylphenol-Polyglykolether
Octanolpolyalkylenglycolether
Octandiol-bis-(polyalkylenglykolether)
Poly(ethylenglykol-ran-propylenglykol)
Poly(ethylenglykol)-*block*-poly(propylenglykol)-*block*-poly(ethylenglykol) und
Poly(propylenglykol)-*block*-poly(ethylenglykol)-*block*-poly(propylenglykol).

8. Lösung nach einem der vorstehenden Ansprüche, **dadurch gekennzeichnet, dass** die mindestens eine wasserlösliche Schwefelverbindung ausgewählt ist aus der Gruppe, umfassend organische, stickstofffreie Thioverbindungen und deren Salze.

9. Lösung nach Anspruch 8, **dadurch gekennzeichnet, dass** die Salze Alkali- oder Erdalkalimetallionen enthalten, ausgewählt aus der Gruppe, umfassend Natrium-, Kalium-, Magnesium- und Calcium.

10. Lösung nach einem der Ansprüche 8 und 9, **dadurch gekennzeichnet, dass** die mindestens eine organische, stickstofffreie Thioverbindung ausgewählt ist aus der Gruppe, umfassend:
3-(Benzthiazolyl-2-thio)-propylsulfonsäure, Natriumsalz
3-Mercaptopropan-1-sulfonsäure, Natriumsalz
Thiophosphorsäure-O-ethyl-bis-(ω-sulfopropyl)-ester, Dinatriumsalz
Thiophosphorsäure-tris-(ω-sulfopropyl)-ester, Trinatriumsalz
Ethylendithiodipropylsulfonsäure, Natriumsalz
Bis-(*p*-sulfophenyl)-disulfid, Dinatriumsalz
Bis-(ω-sulfopropyl)-sulfid, Dinatriumsalz
Bis-(ω-sulfopropyl)-disulfid, Dinatriumsalz
Bis-(ω-sulfohydroxypropyl)-disulfid, Dinatriumsalz
Bis-(ω-sulfobutyl)-disulfid, Dinatriumsalz
Methyl-(ω-sulfopropyl)-disulfid, Natriumsalz
Methyl-(ω-sulfobutyl)-trisulfid, Natriumsalz
O-Ethyl-dithiokohlensäure-S-(ω-sulfopropyl)-ester, Kaliumsalz Thioglykolsäure

11. Lösung nach einem der vorstehenden Ansprüche, **dadurch gekennzeichnet, dass** Säure in der Lösung enthalten ist und dass die Säure ausgewählt ist aus der Gruppe, umfassend Schwefelsäure, Salzsäure, Fluorborsäure und Methansulfonsäure.

12. Lösung nach einem der vorstehenden Ansprüche, **dadurch gekennzeichnet, dass** die Lösung zusätzlich Chloridionen enthält.

13. Lösung nach Anspruch 12, **dadurch gekennzeichnet, dass** die Chloridionen in Form von Natriumchlorid und/oder von Salzsäure zu der Lösung zugegeben worden sind.

14. Lösung nach einem der vorstehenden Ansprüche, **dadurch gekennzeichnet, dass** die Lösung zusätzlich mindestens eine organische, stickstoffhaltige Thioverbindung enthält.

15. Lösung nach Anspruch 14, **dadurch gekennzeichnet, dass** die mindestens eine stickstoffhaltige Thioverbindung ausgewählt ist aus der Gruppe, umfassend:
Thioharnstoff
N-Acetylthioharnstoff
N-Trifluoroacetythioharnstoff
N-Ethylthioharnstoff
N-Cyanoacetylthioharnstoff
N-Allylthioharnstoff
o-Tolylthioharnstoff
N,N'-Butylenthioharnstoff
Thiazolidinthiol-2
4-Thiazolinthiol-2
Imidazolidinthiol-2-(N,N'-Ethylenthioharnstoff)
4-Methyl-2-pyrimidinthiol
2-Thiouracil.

16. Lösung nach einem der vorstehenden Ansprüche, **dadurch gekennzeichnet, dass** die Lösung zusätzlich mindestens eine polymere Phenaziniumverbindung enthält.

17. Lösung nach Anspruch 16, **dadurch gekennzeichnet, dass** die mindestens eine polymere Phenaziniumverbindung ausgewählt ist aus der Gruppe, umfassend:
Poly(6-methyl-7-dimethylamino-5-phenyl-phenaziniumsulfat)
Poly(2-methyl-7-diethylamino-5-phenyl-phenaziniumchlorid)
Poly(2-methyl-7-dimethylamino-5-phenyl-phenaziniumsulfat)
Poly(5-methyl-7-dimethylamino-phenaziniumacetat)
Poly(2-methyl-7-anilino-5-phenyl-phenaziniumsulfat)
Poly(2-methyl-7-dimethylamino-phenaziniumsulfat)
Poly(7-methylamino-5-phenyl-phenaziniumacetat)
Poly(7-ethylamino-2,5-diphenyl-phenaziniumchlorid)
Poly(2,8-dimethyl-7-diethylamino-5-p-tolyl-phenaziniumchlorid)
Poly(2,5,8-triphenyl-7-dimethylamino-phenaziniumsulfat)
Poly(2,8-dimethyl-7-amino-5-phenyl-phenaziniumsulfat)
Poly(7-Dimethylamino-5-phenyl-phenaziniumchlorid)

18. Lösung nach einem der vorstehenden Ansprüche, **dadurch gekennzeichnet, dass** die Lösung zusätzlich mindestens eine polymere Stickstoffverbindung enthält.

19. Lösung nach Anspruch 18, **dadurch gekennzeichnet, dass** die mindestens eine polymere Stickstoffverbindung ausgewählt ist aus der Gruppe, umfassend Polyethylenimin, Polyethylenimid, Polyacrylsäureamid, Polypropylenimin, Polybutylenimin, N-Methylpolyethylenimin, N-Acetylpolyethylenimin und N-Butylpolyethylenimin.

20. Verwendung der Lösung nach einem der Ansprüche 1-19 zur Abscheidung eines Kupferüberzuges.

21. Verwendung der Lösung nach Anspruch 20 zur Abscheidung von Kupfer auf Leiterplattenmaterial.

22. Verwendung nach einem der Ansprüche 20 und 21 zur Herstellung von Kupferüberzügen in Vertikal- und/oder Horizontalmetallisierungsanlagen.

23. Verfahren zum galvanischen Abscheiden von Kupferüberzügen auf Metall- oder Kunststoffoberflächen, umfassend In-Kontakt-Bringen der Oberflächen mit der Lösung nach einem der Ansprüche 1-19 und elektrolytisches Abscheiden von Kupfer auf den Oberflächen.

## Revendications

1. Solution acide aqueuse pour dépôt électrolytique de revêtements de cuivre, ladite solution contenant au moins un composé de polyalcylène glycol et au moins un composé de soufre soluble dans l'eau, **caractérisée en ce que** la solution contient en outre au moins un dérivé d'halogène aromatique ayant la formule générale (I) dans laquelle
R₁, R₂, R₃, R₄, R₅ et R₆ sont chacun indépendamment des radicaux choisis dans le groupe comprenant l'hydrogène, l'aldéhyde, l'acétyle, l'hydroxy, l'hydroxyalkyle ayant 1-4 atomes de carbone, l'alkyle ayant 1-4 atomes de carbone et l'halogène, à condition que le nombre de radicaux R₁, R₂, R₃, R₄, R₅ et R₆ qui sont des halogènes soit compris de 1 à 5 et qu'au moins un des R₁, R₂, R₃, R₄, R₅ et R₆ soit choisi dans le groupe constitué d'hydroxy, aldéhyde, acétyle et hydroxyalkyle ayant 1-4 atomes de carbone, dans lequel la concentration d'au moins un dérivé d'halogène aromatique est comprise de 0,005 à 0,9 mg/l.

2. Solution selon l'une quelconque des revendications précédentes, **caractérisée en ce que** l'aldéhyde est choisi dans le groupe comprenant le formyle (-CHO), le méthylformyle (-CH₂-CHO) et l'éthylformyle (-C₂H₄-CHO).

3. Solution selon l'une quelconque des revendications précédentes, **caractérisée en ce que** l'alkyle est ramifié ou non ramifié et est choisi dans le groupe comprenant le méthyle, l'éthyle, le n-propyle, l'iso-propyle, le n-butyle, l'iso-butyle et le *tert*-butyle.

4. Solution selon l'une quelconque des revendications précédentes, **caractérisée en ce que** l'alkyle est un hydroxyalkyle et qu'il est ramifié ou non ramifié.

5. Solution selon l'une quelconque des revendications précédentes, **caractérisée en ce qu'**au moins un hydroxyalkyle est un hydroxyméthyle.

6. Solution selon l'une quelconque des revendications précédentes, **caractérisée en ce que** ledit au moins un dérivé halogène aromatique est choisi dans le groupe comprenant le
2-chlorobenzaldéhyde
2-chlorophénol
4-chloro-3-méthylphénol
2-chloro-4,5-diméthylphénol
4-chloro-3,5-diméthylphénol
4-chlorophénol
3-chlorophénol
o-chloroacétophénone
alcool de 2-chlorobenzyle
4-bromo-2,6-diméthylphénol
4-bromophénol
alcool de 2,4-dichlorobenzyle
2,6-dibromo-4-méthylphénol
2,5-dichlorophénol
3,5-dibromobenzaldéhyde
acide 2,5-dibromobenzoïque
2,4,6-trichlorophénol
2,3,6-trichlorobenzaldéhyde

7. Solution selon l'une quelconque des revendications précédentes, **caractérisée en ce que** ledit au moins un additif contenant de l'oxygène, à masse moléculaire élevé, est choisi dans le groupe comprenant le:
alcool de polyvinyle
carboxyméthylcellulose
polyéthylène glycol
polypropylène glycol
ester de polyglycol d'acide stéarique
ester de polyglycol d'acide oléique
éther de polyglycol d'alcool de stéaryle
éther de polyglycol de nonylphénol
éther de polyalcylène glycol d'octanol
octanediol-bis-(polyalcylène glycol éther)
poly(éthylène glycol-*ran*-propylène glycol)
poly(éthylène glycol)-*bloc*-poly(propylène glycol)-*bloc*-poly(éthylène glycol) et
poly(propylène glycol)-*bloc*-poly(éthylène glycol)-*bloc*-poly(propylène glycol).

8. Solution selon l'une quelconque des revendications précédentes, **caractérisée en ce que** ledit au moins un composé de soufre soluble dans l'eau est choisi dans le groupe comprenant les composés thio organiques sans azote, et leurs sels.

9. Solution selon la revendication 8, **caractérisée en ce que** les sels contiennent des ions métalliques alcalins ou alcalino-terreux, choisis dans le groupe comprenant le sodium, de potassium, de magnésium et de calcium.

10. Solution selon l'une quelconque des revendications 8 et 9, **caractérisée en ce que** ledit au moins un composé thio organique sans azote est choisi dans le groupe comprenant le
sel de sodium d'acide 3-(benzothiazolyl-2-thio)-propylsulfonique
sel de sodium d'acide 3-mercaptopropane-1-sulfonique
sel de disodium d'acide thiophosphorique-O-éthyl-bis-(ω-sulfopropyl)-ester
sel de trisodium d'acide thiophosphorique-tris-(ω-sulfopropyl)-ester
sel de sodium d'acide d'éthylènedithio-dipropyl-sulfonique
sel de disodium de bis-(*p*-sulfophényl)-disulfure
sel de disodium de bis-(ω-sulfopropyl)-sulfure
sel de disodium de bis-(ω-sulfopropyl)-disulfure
sel de disodium de bis-(ω-sulfohydroxypropyl)-disulfure
sel de disodium de bis-(ω-sulfobutyl)-disulfure
sel de sodium de méthyl-(ω-sulfopropyl)-disulfure
sel de sodium de méthyl-(ω-sulfobutyl)-trisulfure
sel de potassium d'acide O-éthyl-dithiocarbonique-S-(ω-sulfopropyl)-ester
acide thioglycolique

11. Solution selon l'une quelconque des revendications précédentes, **caractérisée en ce que** de l'acide est contenu dans la solution et que l'acide est choisi dans le groupe comprenant l'acide sulfurique, l'acide chlorhydrique, de l'acide fluoroborique, et l'acide méthanesulfonique.

12. Solution selon l'une quelconque des revendications précédentes, **caractérisée en ce que** la solution contient en outre des ions chlorure.

13. Solution selon la revendication 12, **caractérisée en ce que** les ions chlorure ont été ajoutés à la solution sous forme de chlorure de sodium et/ou d'acide chlorhydrique.

14. Solution selon l'une quelconque des revendications précédentes, **caractérisée en ce que** la solution contient en outre au moins un composé thio organique, contenant de l'azote.

15. Solution selon la revendication 14, **caractérisée en ce que** ledit au moins un composé thio contenant de l'azote est choisi dans le groupe comprenant le
thiourée
N-acétylthiourée
N-trifluoroacétyl thiourée
N-éthylthiourée
N-cyanoacétyl thiourée
N-allylthiourée
*o*-tolylthiourée
N,N'-butylène thiourée
thiazolidine thiol-2
4-thiazoline thiol-2
imidazolidine thiol-2-(N,N'-éthylène thiourée)
4-méthyl-2-pyrimidine thiol
2-thiouracil

16. Solution selon l'une quelconque des revendications précédentes, **caractérisée en ce que** la solution contient en outre au moins un composé de phénazinium polymère.

17. Solution selon la revendication 16, **caractérisée en ce que** ledit au moins un composé de phénazinium polymère est choisi dans le groupe comprenant le:
poly(6-méthyl-7-diméthylamino-5-phényl-phénazinium sulfate)
poly(2-méthyl-7-diéthylamino-5-phényl-phénazinium chlorure)
poly(2-méthyl-7-diméthylamino-5-phényl-phénazinium sulfate)
poly(5-méthyl-7-diméthylamino-phénazinium acétate)
poly(2-méthyl-7-anilino-5-phényl-phénazinium sulfate)
poly(2-méthyl-7-diméthylamino-phénazinium sulfate)
poly(7-méthylamino-5-phényl-phénazinium acétate)
poly(7-éthylamino-2,5-diphényl-phénazinium chlorure)
poly(2,8-diméthyl-7-diéthylamino-5-*p*-tolyl-phénazinium chlorure)
poly(2,5,8-triphényl-7-diméthylamino-phénazinium sulfate)
poly(2,8-diméthyl-7-amino-5-phényl-phénazinium sulfate)
poly(7-diméthylamino-5-phényl-phénazinium chlorure)

18. Solution selon l'une quelconque des revendications précédentes, **caractérisée en ce que** la solution contient en outre au moins un composé d'azote polymère.

19. Solution selon la revendication 18, **caractérisée en ce que** ledit au moins un composé d'azote polymère est choisi dans le groupe comprenant le polyéthylène imine, le polyéthylène imide, amide d'acide polyacrylique, polypropylène imine, polybutylène imine, N-méthyl polyéthylène imine, N-acétyl polyéthylène imine, N-butyl polyéthylène imine.

20. Utilisation de la solution selon l'une quelconque des revendications 1-19 pour déposer un revêtement de cuivre.

21. Utilisation de la solution selon la revendication 20 pour déposer du cuivre sur un matériau de carte à circuit imprimé.

22. Utilisation selon l'une quelconque des revendications 20 et 21 pour produire des revêtements de cuivre dans des lignes de plaquage, verticales et/ou horizontales, dotées de convoyeurs.

23. Procédé de déposition électrolytique de revêtements de cuivre sur des surfaces métalliques ou plastiques, comprenant la mise en contact des surfaces avec la solution, selon l'une quelconque des revendications 1-19, et le dépôt électrolytique de cuivre sur les surfaces.
